

## UNITED STATES PATENT OFFICE

2,143,803

## PROCESS FOR BLEACHING RAW STOCK COTTON

Edwin P. Sherman, High Point, N. C., assignor to  
The Geo. E. Sherman Company, Inc., Brooklyn,  
N. Y., a corporation of New York

No Drawing. Original application March 11, 1937,  
Serial No. 130,417. Divided and this applica-  
tion March 2, 1938, Serial No. 193,604

## 2 Claims. (Cl. 8—108)

This invention relates to bleaching processes, more particularly to a process for bleaching raw stock cotton, and is a division of my co-pending application for patent filed March 11, 1937, Serial 5 Number 130,417.

Standard bleaching processes are relatively complicated and lengthy as, for example, the bleaching of cotton yarn, which involves substantially seven steps, as follows,—boiling in caustic, 10 as 2% caustic soda, 1% silicate and 1% sulphonated oil or the like, dropping the above bath and washing in hot water, dropping and running through hypochlorite solution  $\frac{1}{2}$  to 2 Tw., dropping and washing in warm water, dropping and 15 souring in a hydrochloric acid or sulphuric acid solution or the like, dropping and washing in warm water, dropping and washing in water to which is added bluing.

An object of this invention is to provide a 20 bleaching process which is much shorter than standard processes, and involves fewer steps.

Another object is to provide a bleaching process employing a compound containing oxygen and chlorine which process will inhibit the characteristic action of the chlorine upon the fibers without interfering with the action of the nascent 25 oxygen.

Still another object is to provide an improved 30 bleaching process which will be efficient, even if the material to be bleached contains insoluble oils.

Another object is to provide a bleaching process which will leave the material free of oil stains, chafe marks and so-called niger beads.

35 Yet another object is to provide a bleaching process which is considerably less expensive than most standard bleaching processes for like material.

Other objects and advantages of the invention 40 will be apparent during the course of the following detailed description thereof.

In the sodium hypochlorite-buffer hereinafter referred to, the buffer may be glues, saponified and/or emulsified fats and oils, sulphonated oils, dextrines, glucose, sugar, fatty alcohols, alkali and alkaline salts.

The sodium hypochlorite and buffer may be mixed together in substantially the following proportions:—

| Sodium hypochlorite | Per cent<br>by weight |
|---------------------|-----------------------|
| Buffer              | 5                     |

45 However, the percentages of sodium hypochlorite may vary between 95% and 99% while the percentages of buffer may vary between 1% and 5%.

As required, the sodium hypochlorite-buffer mixture may be employed already mixed, since

it has been found that this mixture does not lose strength even after being kept for a considerable period.

For bleaching raw stock cotton, the same is, preferably, treated by boiling for one hour in a 5 5% caustic soda bath, and is then given a hot rinse (180° F. to boiling) for substantially one-half hour after which it is introduced to a bath which includes:—

|                                    | Percent |
|------------------------------------|---------|
| Soda ash                           | 10      |
| Sodium stearate                    | 2       |
| Sodium hypochlorite-buffer mixture | 1       |
|                                    | 8       |

In this treatment of raw stock cotton, the bath last mentioned is maintained at substantially 110° F. for one hour, whereupon the temperature is raised to the boiling point and boiling maintained for substantially forty-five minutes. Thereupon, this bath is dropped, and the material given a good rinse at 120° F., using 1% sodium 15 stearate and bluing, as desired, in the rinse water. After this last rinse, the material may be 20 extracted.

With the treatment described, the chlorine does not attack the material being bleached, due 25 to the proportions of buffers employed and the temperatures maintained.

Various changes may be made to the forms of the invention herein described, without departing from the spirit of the invention or the scope 30 of the claims.

What is claimed is:

1. A bleaching process for raw stock cotton, which consists in boiling said cotton in a caustic 35 soda solution, hot rinsing said material for substantially thirty minutes, subjecting said cotton to a bath including soda ash, sodium stearate, sodium hypochlorite and a buffer, said bath being at a temperature of substantially 110° F., maintaining said temperature of said bath for substantially one hour, raising said temperature of 40 said bath to the boiling point and boiling for substantially forty-five minutes, dropping said bath and rinsing said cotton.

2. A bleaching process for raw stock cotton, which consists in boiling said cotton in a caustic soda solution, hot rinsing said material for substantially thirty minutes, subjecting said cotton to a bath including 2% soda ash, 1% sodium stearate, 8% sodium hypochlorite buffer mixture, 50 said bath being at a temperature of substantially 110° F., maintaining said temperature of said bath for substantially one hour, raising said temperature of said bath to the boiling point and boiling for substantially forty-five minutes, dropping 55 said bath and rinsing said cotton.

EDWIN P. SHERMAN.